

(No Model.)

3 Sheets—Sheet 1.

R. O. LORENZ.

APPARATUS FOR PRODUCING ZINC AND LEAD BY ELECTROLYSIS.

No. 559,729.

Patented May 5, 1896.



Witnesses.

*Dennis Sumbly,  
Robert Everett.*

Inventor.

*Richard O. Lorenz.*

By Attorney  
*James L. Morris*

(No Model.)

3 Sheets—Sheet 2.

R. O. LORENZ.

APPARATUS FOR PRODUCING ZINC AND LEAD BY ELECTROLYSIS.

No. 559,729.

Patented May 5, 1896.

Fig II.



Fig III.



Witnesses.

Dennis Sumbry.  
Robert Everett.

Inventor.

Richard O. Lorenz.

By Attorney.

James G. Morris.

(No Model.)

3 Sheets—Sheet 3.

R. O. LORENZ.

APPARATUS FOR PRODUCING ZINC AND LEAD BY ELECTROLYSIS.

No. 559,729.

Patented May 5, 1896.



*Witnesses.*  
Robert Elliott,  
Thos. A. Grun

*Inventor:*  
Richard O. Lorenz.  
By Attorney,  
*James L. Morris.*

# UNITED STATES PATENT OFFICE.

RICHARD OTTOKAR LORENZ, OF GÖTTINGEN, GERMANY.

## APPARATUS FOR PRODUCING ZINC AND LEAD BY ELECTROLYSIS.

SPECIFICATION forming part of Letters Patent No. 559,729, dated May 5, 1896.

Application filed January 4, 1895. Serial No. 533,849. (No model.)

*To all whom it may concern:*

Be it known that I, RICHARD OTTOKAR LORENZ, a subject of the Grand Duke of Saxe-Weimar-Eisenach, and a resident of Göttingen, German Empire, am in possession of an invention for an Apparatus for the Production of Zinc and Lead by Electrolysis of the Melted Chlorids; and I do hereby declare the nature of the said invention and in what manner the same is to be performed to be particularly described and ascertained in and by the following statement thereof—that is to say:

This invention has for its object to effect a rational working of ores containing zinc and lead, in particular of so-called "mixed" ores, of residue alloys containing zinc and lead and the like. This is effected by converting the compounds containing zinc and lead into chlorids, which are subjected to an electrolytic process under the influence of heat. The production of the chlorids is effected according to the usual methods, the use of which will of course depend upon the nature of the raw materials treated.

When treating zinc ores, lead ores, and mixed zinc and lead ores, they are roasted in the usual manner for conversion into oxids. If the ores are mainly zinc ores, and consequently contain but little lead, and possibly a small quantity of silver, cadmium, &c., they are lixiviated directly with hydrochloric acid of medium strength. The lyes then contain mostly zinc chlorid, as also small quantities of chlorids of lead, silver, cadmium, &c., together with the calcium and magnesium chlorids that may be present. If an excess of hydrochloric acid has been used, the lye will of course also contain iron and aluminium chlorids. As these latter would interfere with the electrolytic action they are precipitated by the addition of roasted ore or zinc residues. The lyes thus purified after having been clarified are evaporated to dryness and melted.

If, on the other hand, the ores are mainly lead ores, either pure or containing zinc, and consequently contain so much lead that on lixiviating them by means of hydrochloric acid insoluble lead chlorid would be precipitated, the roasted material is lixiviated with dilute acetic acid, and hydrochloric-acid gas is led through the ace-

tate solution, or concentrated acid is added thereto until the whole of the lead and silver are precipitated as chlorids. The clarified lyes are then decanted and heated for the separation of iron and alumina, and then again clarified and decanted. The discharged lyes, which again contain much free acetic acid, are used for the lixiviation of fresh quantities of roasted ore, and this process is repeated until all the acetic acid has combined with zinc. For regenerating the acetic acid the zinc is made to combine with hydrochloric-acid gas introduced for that purpose, and the lye is then distilled to dryness. The distillate, condensed in the usual manner, now contains the whole of the acetic acid, which can be used again for lixiviating fresh quantities of roasted ore.

It is evident that by a suitable mixture of the ores either before roasting or after roasting the one or the other process of lixiviation can be employed, according as circumstances may require.

When treating alloys or waste containing zinc and lead—such as zinc-dust, zinc residues, muffle residues, &c.—the raw material is treated by the one or the other of the above-described processes, according to the composition thereof.

When zinc chlorid is treated, such as is obtained as by-product in various technical processes, such as in color-manufactories, it can be at once melted and subjected to electrolysis.

For carrying out the electrolytic process the apparatus shown diagrammatically on the accompanying drawings illustrates my invention.

Figure 1 shows a sectional view of the apparatus. Fig. 2 shows the arrangement of the electrodes; Fig. 3, a plan view of the cover and of the electrodes, in which the connecting-plate for the electrodes is removed. Fig. 4 is a vertical section of a retort for recovering muriatic acid from the chlorin.

In the inclined brickwork firing-chamber A is contained a vessel B for containing the melted electrolyte. When constructed on a small scale, this vessel may be made of porcelain or of refractory clay containing a large percentage of kaolin and as free as possible from iron. When constructed on a large

scale, it is built of enameled bricks, which are bound together by a suitable binding material consisting mainly of kaolin.

The vessel B, of whatever material, is enclosed in an iron casing b for preventing the penetration of combustion-gases into the electrolyte. For protecting the casing b against the action of the combustion-gases it can be provided externally with a coating of clay and the like, as more clearly shown at b' in Fig. 1.

The vessel A is closed at top by means of a cover C of clay. For carrying off the gases formed by the electrolytic action a lateral tubular branch D is provided, by means of which the gases are led into the earthenware pipe E, in which they are conducted to wherever required.

At the lower end the vessel A is tapered to form a pocket G, terminating in a pipe F, the end of which terminates in a discharging device H.

The section of the vessel B can be of any shape, but would preferably be made circular or elliptic. In the accompanying drawings an elliptic section has been chosen, as seen in Fig. 3.

The electrodes are fixed in the cover C, all chinks being hermetically sealed. The electrodes at their upper ends are united by a plate P, formed of any suitable fireproof material—such as fireproof clay, for example. If the aforesaid chlorids are subjected to electrolysis in an impure state—for instance, in case they should still contain a certain quantity of water or of organic substances—such impurities will also be decomposed by the action of the current. In that case, besides the products resulting from the decomposition of the chlorids, other bodies, and especially gases, will be generated at both electrodes. If these gases be permitted to intermingle in *statu nascendi*, it can easily happen that they reunite in consequence of their natural affinity and the high temperature of the electrolyte. Such reunion not only causes explosions within the electrolyte, and in consequence violent foaming, which much disturbs the regular process, but also a not inconsiderable loss of energy, because the bodies formed by the reunion of these products—*i. e.*, principally hydrochloric acid and water—are thus subjected to electrolytic decomposition over and over again. This difficulty is mainly overcome by the inclined position of the retort containing the electrolyte and by the peculiar shape of the electrodes. The anode is placed above the middle of the retort and the cathode below. Moreover both electrodes are so formed that the gas generated at the bottom side of the anode can freely pass through or around to the upper side and that the metal precipitated at the cathode can freely sink through or around the electrode to the bottom of the vessel. This purpose is achieved by forming the electrodes of intersecting parts having numerous openings between the intersections,

so that in appearance they resemble network or grates, as shown in Figs. 1 and 2.

In the accompanying drawings, Fig. 3 shows the electrodes composed each of three carbon bars K K' K<sup>2</sup> and L L' L<sup>2</sup> of circular section. By these means—*i. e.*, the inclined position of the retort and the grate-shaped electrodes—sufficient separation of the products of decomposition is arrived at, although the electrodes present a considerable surface to each other and the distance between them is comparatively small.

The carbons K K' K<sup>2</sup> serve as anodes and L L' L<sup>2</sup> as cathodes.

Through the branch D can be introduced a porcelain tube M, serving to charge the vessel A with the melted electrolyte. The gases (chlorin) developed at the anodes rise up along the same, in consequence of the inclined position thereof, in the space R between the anodes and the sides of the vessel and pass through branch D into the pipe E, which leads them to wherever required.

At the cathodes L L' L<sup>2</sup> the metal is separated in a molten condition and drips in melted balls into the pocket G, where it is collected and discharged from time to time.

The molten mass subjected to electrolysis always consists of a mixture of lead chlorid and zinc chlorid, with or without addition of the other chlorids above mentioned, of which silver chlorid is of particular importance. According to its origin the zinc or the lead can predominate in the mass.

By means of the above-described process of lixiviation by acetic acid it is, no doubt, possible to separate the chlorids of zinc and lead from each other, so that the chlorids of each of the metals could be separately electrolyzed; but in most cases it has been proved advantageous to subject a mixture of the chlorids to electrolysis and, if the chlorids should have been obtained separately, to mix them together before electrolyzing them. The mass from the melting-crucibles is either introduced liquid into the decomposing-furnace or, after cooling, it can be introduced in pieces and melted down therein at a moderate temperature. It is advantageous to fill the furnace to about two-thirds of its capacity.

In carrying out the electrolysis a current having a tension of from 0.4 to one volt is used. Special attention requires to be paid during the process to the regulation of the temperature. It must be kept above the melting-point of the mixture of zinc and lead chlorids and of the zinc, (or the lead,) but below the boiling-point of the zinc chlorid—that is to say, between the limits of 450° to 680° centigrade. As soon as the entire mass is melted the electric circuit is closed. The chlorin developed at the anode rises, as described, and is led off by the pipe E. It may be suitably stored in gas-holders and can be utilized in any manner desired. The metal separated at the cathode drops in spherical form from the same and rolls down into the pocket G,

whence it is tapped off. During the electrolysis fresh material is introduced through the pipe M, according as the charge is consumed, so that the working is continuous. During the electrolysis of the mass the metals contained therein do not separate simultaneously, but one after the other, the separation of the separated metals being dependent upon the tension of the current employed at the time, as also upon the proportion of the several constituents. This fact enables the fractional separation to be effected, and consequently a separation of the several metals. There will be first separated silver and then lead; but as the silver only exists in small quantities and does not melt at the temperature of 450° to 680° centigrade the electrolysis is at the first stage of the process conducted in such manner that simultaneously with the silver a certain quantity of lead is separated, which forms with the silver an easily-fusible alloy. This alloy then drops from the electrodes into the pocket. During this stage samples should be frequently taken and examined as to percentage of silver. As soon as silver ceases to appear in appreciable quantities the lead containing silver is tapped off. As a second fraction of the electrolysis pure lead is separated. After tapping this off the metal now discharged consists of an alloy of the last residues of the lead with the other metals present with the exception of zinc. The electrolyte then only consists of pure zinc chlorid, from which lastly chemically pure zinc is obtained. The zinc and lead obtained by the electrolysis are absolutely pure—that is to say, of one hundred per cent.

The periods of time within which the several metals are separated and consequently the discharge must take place are determined by an analysis of the particular product employed and depend upon the nature of the electrolyte.

During the process the tension of the current is made to vary. For the separation of the lead a tension of 0.4 to 0.5 of a volt is sufficient. During the separation of the zinc a tension of from 0.8 to one volt is employed.

In some cases it is desirable to regulate the electrolytic process. This is effected by means of suitable additions which influence the melting temperature and the conducting power of the electrolyte. As such additions I may use, among others, sodium chlorid, potassium chlorid, magnesium chlorid, calcium chlorid, sodium fluorid, fluor-spar, and the like.

Certain kinds of commercial zinc chlorid, in particular those which proceed from color-manufactories, cannot be dehydrated by melting only, and contain in addition to organic substances in many cases ammonium chlorid. If such zinc chlorid is subjected to electrolysis, then at the commencement thereof there will escape oxygen, chlorin, hydrochloric acid, and ammonia, which cause an objectionable frothing of the melt combined with the defective separation of the metals. For preventing

this disadvantage an addition of litharge, red lead, zinc oxid, and other metallic oxids or super-oxids is employed during the melting 70 or before the commencement of electrolysis.

The addition of the metallic oxid or super-oxid in the manner set forth is for the purpose of neutralizing impurities which may be present in the electrolyte, such as ammonium 75 chlorid or free muriatic acid. Such impurities, as well as water, if present, may cause the electrolyte to foam, as they cause a secondary decomposition by which gases—such as hydrogen, chlorin, and oxygen—are given off. 80 These gases form bubbles which rise and cause foam. Being in a nascent state they are liable also to unite by their affinity and again mingle with the electrolyte, from which they are again evolved. 85

The chemical action may be stated as follows: If the electrolyte contains ammonium chlorid, the addition of oxid of lead and the resulting combinations may be stated by the equation: 90



If oxid of zinc is used, the formula will be:



Thus the ammonium chlorid is decomposed by these oxids and combined with the electrolyte.

If organic matter is present, a superoxid of lead will destroy it. If free muriatic acid 100 or hydrochloric-acid gas is present, by which hydrogen would be formed at the cathode, the metallic oxid will convert the muriatic or hydrochloric acid to the chlorid of the metal used. This is expressed by the following 105 equations:



By adding chlorid of lead to an electrolyte strongly charged with chlorid of zinc and retaining water the latter will be removed by physical displacement in accordance with the natural law. 115

The chlorin developed of the anodes is collected in suitable gas-holders, and is led thence through vertical, horizontal, or inclined clay retorts filled with coke, charcoal, or anthracite and heated to a low red heat, steam being at the same time forced in. The apparatus for this purpose is shown in Fig. 4 and is as follows: To obtain muriatic acid from the chlorin, a retort heated from the outside and made of fireproof material can be used. That 125 which seems to fulfill all conditions best is an upright retort heated from the outside by means of generator-gas, as represented in Fig. 4. The apparatus, as represented in the drawings, consists of an upright retort S, 130 made of fireproof material, which is bricked up in such a manner that it may be heated by means of generator-gas, inducted by means of pipes z into the fire-space. These retorts

have a movable cover *s*, which by means of an appropriate locking device is fastened during the operation. The retort is filled from above with coke and is then heated to a medium red heat. Chlorin is then introduced by means of pipe *T*. At the same time steam is admitted into the retort by means of steam-pipes *W* and *w*. The gaseous products originating from this combination of coke, steam, and chlorin—such as muriatic acid, oxid of carbon, and carbonic acid—are led through pipe *U* into condensing vessels *V*, (the drawings show only one of these vessels,) where the muriatic acid condenses. A reaction will then take place under these conditions between the carbon, water, and chlorin according to the following formula:

1.  $C + H_2O + Cl_2 = 2HCl + CO$ .
2.  $C + 2H_2O + 2Cl_2 = 4HCl + CO_2$ .

Here will consequently pass away from the retort together with the hydrochloric-acid gas a mixture of carbonic acid and carbonic oxid. The hydrochloric acid is condensed out of this mixture in the ordinary condensing apparatus and the chlorin absorbed by water in the ordinary manner.

By the above-described method it is ren-

dered possible to convert any quantity of 30 chlorin in a very short time into absolutely pure hydrochloric acid.

The carbonic-oxid and carbonic-acid gases on issuing from the hydrochloric-acid-condensing apparatus are collected in gas-holders 35 and may be utilized in any desired manner.

Having now particularly described and ascertained the nature of this invention and in what manner the same is to be performed, I declare that what I claim is—

An apparatus for practicing the described process comprising a retort, or vessel, which is oval in cross-section, said retort being so inclined that the plane coinciding with its major axis and perpendicular to the sides of 45 said vessel is inclined at an angle with a vertical line, anodes and cathodes sealed hermetically in said retort and having a like inclination, the anodes being arranged over, or above the said plane and the cathodes on the 50 under side of and below said plane, said electrodes being formed of intersecting parts having openings between the intersections, substantially as described.

RICHARD OTTOKAR LORENZ.

Witnesses:

LUDWIG KOENIG,

MAX WAGNER.